

1

3,159,510

**HIGH-SPEED QUENCHING COMPOSITION**  
 Irving Rozalsky, East Alton, and Curtis L. Early, Alton,  
 Ill., assignors to Shell Oil Company, New York, N.Y.,  
 a corporation of Delaware  
 No Drawing. Filed Feb. 23, 1962, Ser. No. 175,339  
 10 Claims. (Cl. 148—29)

This invention relates to improved high-speed quenching oil compositions for use in the metallurgical industries and to the method of quenching metals therewith.

In the process of hardening metals such as steel, it is common practice to use as the quenching medium water, oil or compressed air, according to the type of steel. Recently salts or aqueous solutions of salts have also been used for this purpose, but these have the disadvantage that they solidify or deposit solids on cooling to room temperature. Fatty oils, especially rapeseed oil, are used as quenching oils, but these have been gradually superseded by mineral quenching oils. It has also been proposed to harden and temper steels using baths containing naphthalene mono- or disulfonic acids or salts thereof or anthracene mono- or disulfonic acids or salts thereof. Sulfonic acids or their salts are mixed with water or oil to form the treating bath and the oils generally used are linseed oil, cotton seed oil and other fatty substances.

Quenching compositions of the above types are defective in a number of respects among which are that water or emulsion quenching causes stress and strains in the metal such as steel which results in warping and cracking thereof, rendering the metal unusable. Oil quenching, although essential obviating this objectionable characteristic of water or emulsion quenching compositions, tend to leave adherent deposits on quenched metal surfaces which must be removed by relatively expensive buffing or machining operations prior to further processing of the metal. This, plus the fact that oil quenching is expensive and the life of such oil is short because of thermal and oxidation deterioration, thereby requiring continuous replacement with fresh oils, presents a pressing problem to the industry.

An object of the present invention is an improved process for quenching metals. A further object is to provide a quenching oil composition of superior speed and stability. Another object is to provide a quenching oil composition capable of producing bright quenched metal surfaces. Still other objects will be apparent from the following description of the invention.

The above objects may be attained in accordance with the present invention by quenching a metal in a thermally and oxidatively stable mixture of particular petroleum fractions which contains a critical amount within the range of from about 0.1% to about 2%, preferably between 0.2% and 0.5% by weight each of an additive mixture comprising (A) a non-ash forming oil-soluble N—C<sub>10-24</sub> acyl sarcosine and nitrogen-base salts or esters thereof and (B) an oil-soluble alkali or alkaline earth metal petroleum sulfonates.

By the particular petroleum mixture is meant a blend of 50-95% (preferably 60-70%) of (1) a mineral oil fraction in the viscosity range of 80-250 SUS at 100° F., a viscosity index of at least 90, preferably between 95 and 120 and an aromatic content of at least 15%, preferably between 30 and 60%, such as a 100 SUS at 100° F. HVI neutral or 250 SUS at 100° F. HVI neutral and the balance of the blend being (2) a highly refined medium VI (70-80 VI) light mineral oil such as a spray base oil or transformer oil in the viscosity range of from 40-100 SUS at 100° F. and/or a heavy residue fraction such as a 150-210 bright stock or an asphalt or derivatives thereof.

The surprising discovery made resides in the fact that both the mineral oil blend and the additive mixture of the

2

present invention exert a profound effect on both the quenching speed and surface brightness of the metal being treated. Thus using a conventional or ordinary quenching oil such as described in U.S. Patents 2,866,729, 2,485,103 or 2,340,724 with the additives of the present invention taken singly or in combination results in poor quick-quenching and only fair surface brightness.

The first additive (A) namely N—C<sub>10-24</sub> acyl sarcosines and derivatives thereof have the general Formula I



where R is a C<sub>10-24</sub> saturated or unsaturated alkyl radical, preferably a C<sub>19-24</sub> unsaturated alkyl radical, and X is the same as R or is a hydrogen or is an amine, preferably a heterocyclic amine. Thus R may be decyl, tetradecyl, dodecyl, tetradecenyl, hexadecenyl, oleyl, ricinoleyl radicals and the amine may be a C<sub>20-18</sub> alkyl amine such as mono- or dioleoyl, dodecyl, tetradecyl, hexadecyl, octadecyl and octadecenyl amines; heterocyclic amines such as substituted imidazolines having the Formula II



where R' is the same as R in Formula I. Examples of N-acyl sarcosines used as quenching speed additive and surface brighteners are illustrated by the following: N-lauroyl sarcosine, N-stearoyl sarcosine, N-caproyl sarcosine, N-myristoyl sarcosine, N-oleoyl sarcosine, N-palmitoyl sarcosine, and N-archidoyl sarcosine, amine salts of such acid as monodecylamine, didecylamine, monotetradecylamine, ditetradecylamine, monoctadecylamine, dioctadecylamine, 1-hydroxyethyl-1-undecylimidazoline, 1-hydroxyethyl-2-heptadecylimidazoline and 1-hydroxyethyl-2-heptadecylimidazoline salts of N-lauroyl sarcosine or N-cocooyl or N-oleoyl sarcosine or N-stearyl sarcosine, particularly preferred compounds are the free acids such as N-oleoyl sarcosine, octadecylamine salts of N-oleoyl sarcosine and 1-hydroxyethyl-2-heptadecenyl imidazoline salt of N-oleoyl sarcosine. The esters include the N—C<sub>20-24</sub> acyl sarcosinates of C<sub>8-20</sub> alkanols such as octyl, decyl, dodecyl and octadecyl alcohols, e.g., N-oleoyl sarcosinate of octyl alcohol, N-oleoyl sarcosinate of octadecyl alcohol. Mixtures of the free acid, ester or amine salts may be used such as a mixture of N-oleoyl sarcosine and 1-hydroxyethyl-2-heptadecenyl imidazoline salt of N-oleoyl sarcosine.

The other essential additive (B) is an oil-soluble alkali metal and/or alkaline earth petroleum sulfonate. These sulfonates are well known in the art and are prepared by reacting a mineral oil with concentrated or fuming sulfuric acid to form oil-soluble sulfonic acids which are then recovered by treatment with an alkali metal base such as sodium hydroxide or potassium hydroxide or with calcium or barium hydroxide or carbonates followed by extraction. These oil-soluble soaps are available as 30% to 70% concentrates in mineral oil.

Although sulfonates are known quenching oil additives because of their ability to improve the speed of quenching, their use has been limited because of their adverse effect on surface finish. In combination with N—C<sub>10-24</sub> acyl sarcosines the sulfonates do not detract from the surface brightness and finish and improve the overall speed of the quenching process.

The oil base blend which is a critical feature of the invention must have thermal and oxidative resistant properties capable of meeting the requirements desired in a quenching oil. Thus the oil of part (1) of the blend must be high viscosity index oil (90-120 VI) in the viscosity range of 80-250 SUS at 100° F., preferably 100-150 SUS at 100° F. and an aromatic content of 15-60%. Such oils

may be illustrated by a HVI 100 neutral having the following properties (Ia):

|                           |      |
|---------------------------|------|
| Gr., API                  | 31.6 |
| Color, NPA                | +1   |
| Flash, ° F.               | 370  |
| Pour point, ° F.          | 0    |
| Viscosity at 100° F., SUS | 103  |
| Viscosity index           | 90   |
| Aromatic, percent         | 15.5 |
| Naphthenes, percent       | 68.9 |
| Paraffins, percent        | 15.6 |

The petroleum fractions of (2) may be illustrated by a mineral spray oil (IIa) of viscosity 45-80 SUS at 100° F., a viscosity index of 70-80 and having 14.7% aromatics, 85.2% naphthenes and 0.1% paraffins or refined transformer oil and the heavy oils (IIc) may be illustrated by 150 HVI bright stock, 170 HVI bright stock having a viscosity index of 90-110 or propane asphalt, petroleum resins, asphaltenes, short residues, etc. Oil blends which are particularly useful are:

|                                                                      |  |
|----------------------------------------------------------------------|--|
| (A) 60% HVI 100 neutral (Ia)                                         |  |
| 30% transformer oil (100 SUS, 100° F., PP, ° F.<br>-60, Color NPA 1) |  |
| 10% unfiltered HVI 150 Bright Stock (VI 95)                          |  |
| (B) 60% HVI 100 neutral (Ia)                                         |  |
| 30% Spray base oil (IIa 45 SUS at 100° F.)                           |  |
| 10% unfiltered HVI 150 Bright Stock                                  |  |
| (C) 95% HVI 100 neutral (Ia)                                         |  |
| 5% propane asphalt                                                   |  |
| (D) 50% HVI 100 neutral (Ia)                                         |  |
| 40% Spray base oil (80 SUS at 100° F.)                               |  |
| 10% Bright Stock (150 neutral)                                       |  |
| (E) 90% HVI neutral (Ia)                                             |  |
| 10% transformer oil                                                  |  |

The compositions of the present invention which contain as the essential additives N-acyl sarcosines and derivatives thereof and alkali metal petroleum sulfonates can be further improved with respect to oxidation stability by addition thereto of from 0.01% to 2%, preferably from 0.1% to 2%, of polymeric ashless dispersants such as nitrogen-containing polymers described in U.S. Patents 2,737,496, 2,839,512, 2,889,282, 2,944,974, or British 808,665 or polyhydric polymeric compounds described in U.S. Patents 2,800,450-2. Polymers of this type having a molecular weight of from 20,000-800,000 can be illustrated by copolymer of lauryl methacrylate/diethylaminoethyl methacrylate, copolymer of 2-methyl-5-vinylpyridine/lauryl methacrylate/stearyl methacrylate, copolymer of 2-methyl-5-vinylpyridine/lauryl methacrylate/stearyl methacrylate/methyl methacrylate, copolymer of vinyl pyrrolidone/lauryl methacrylate, hydrolyzed copolymer of  $C_{10-18}$  alpha-olefin/vinyl acetate. Also desirable is the presence of small amounts (0.1-1%) of phenolic antioxidants such as mono- or bisphenols, preferably phenols which contain at least one tertiary alkyl radical. Alkyl phenols of this type include

2,4,6-triethyl, tributyl, trioctyl,  
2,4-di-tert-butyl-6-methyl,  
2,6-di-tert-butyl-4-methyl,  
2,4,6-di-tert-butyl-  
2,6-dicyclohexyl-4-methyl,  
2,6-dimethyl-4-cyclohexylphenols,  
2,6-di-tert-butyl-  
2,2-di-tert-butyl-  
2,6-tert-butylcyclohexyl,  
2-methyl-6-tert-butyl-4-methylphenols.

The alkyl bisphenols include

1,1-bis-(2-hydroxy-3-tert-butyl-5-methylphenyl)-methane;  
bis(2-hydroxy-3-tert-butyl-5-methylphenyl)ethane;  
1,1-bis(2-hydroxy-3-tert-butyl-5-methylphenyl)propane;  
bis(2-hydroxy-3-tert-butyl-5-methylphenyl)butane;  
bis(2-hydroxy-3-tert-butyl-5-methylphenyl)isobutane;

1,1-bis(2-hydroxy-5-tert-butyl-3-methylphenyl)methane;  
bis(2-hydroxy-5-tert-butyl-3-methylphenyl)ethane;  
1,1-bis(2-hydroxy-5-tert-butyl-3-methylphenyl)propane;  
1,1-bis(2-hydroxy-5-tert-amyl-3-methylphenyl)butane;  
1,1-bis(2-hydroxy-5-tert-amyl-3-methylphenyl)-isobutane; etc.

The 2,4,6-trialkyl phenols containing two tertiary alkyl groups in the 2,4- or 2,6-positions are preferred, such as 2,4-di-tert-butyl-6-methyl-, 2,6-di-tert-butyl-4-methylphenol or 2,6-di-tert-butyl-4-methylophenol or 4,4'-methylene bis(2,6-di-tert-butylphenol).

The following compositions illustrates the invention.

|    |                                  |             |
|----|----------------------------------|-------------|
| 15 | Composition I:                   | Percent wt. |
|    | N-oleoyl sarcosine               | 0.2         |
|    | Sodium petroleum sulfonate       | 0.4         |
|    | 2,6-di-tert-butyl-4-methylphenol | 0.1         |
|    | Base oil blend (A)               | Balance     |

|    |                                                                                           |         |
|----|-------------------------------------------------------------------------------------------|---------|
| 20 | Composition II:                                                                           |         |
|    | N-oleoyl sarcosine                                                                        | 0.25    |
|    | Sodium petroleum sulfonate                                                                | 0.4     |
|    | 2,6-di-tert-butyl-4-methylphenol                                                          | 0.1     |
|    | Copolymer of lauryl methacrylate (90)/diethylamine ethyl methacrylate (10) (M.W. 600,000) | 0.5     |
|    | Base oil blend (A)                                                                        | Balance |

|    |                            |         |
|----|----------------------------|---------|
| 30 | Composition III:           |         |
|    | N-oleoyl sarcosine         | 0.2     |
|    | Sodium petroleum sulfonate | 0.5     |
|    | Base oil blend (A)         | Balance |

|    |                                                                                    |         |
|----|------------------------------------------------------------------------------------|---------|
| 35 | Composition IV:                                                                    |         |
|    | N-oleoyl sarcosine                                                                 | 0.3     |
|    | Potassium petroleum sulfonate                                                      | 0.5     |
|    | Hydrolyzed copolymer of $C_{16-18}$ alpha-olefin/vinyl acetate (3:1) (M.W. 27,000) | 1       |
|    | Base oil blend (D)                                                                 | Balance |

|    |                                                              |         |
|----|--------------------------------------------------------------|---------|
| 40 | Composition V:                                               |         |
|    | 1-hydroxyethyl-2-heptadecenyl imidazoline N-oleoyl sarcosine | 0.2     |
|    | Sodium petroleum sulfonate                                   | 0.4     |
|    | Base oil blend (A)                                           | Balance |

|    |                                   |         |
|----|-----------------------------------|---------|
| 45 | Composition VI:                   |         |
|    | Octadecylamine N-oleoyl sarcosine | 0.5     |
|    | Potassium petroleum sulfonate     | 0.8     |
|    | Base oil blend (B)                | Balance |

|    |                                  |         |
|----|----------------------------------|---------|
| 50 | Composition VII:                 |         |
|    | N-lauroyl sarcosine              | 0.2     |
|    | Sodium petroleum sulfonate       | 0.4     |
|    | 2,6-di-tert-butyl-4-methylphenol | 0.1     |
|    | Base oil blend (A)               | Balance |

|    |                                                                                    |         |
|----|------------------------------------------------------------------------------------|---------|
| 55 | Composition VIII:                                                                  |         |
|    | N-cocoyl sarcosine                                                                 | 0.3     |
|    | Calcium petroleum sulfonate                                                        | 0.5     |
|    | Hydrolyzed copolymer of $C_{16-18}$ alpha-olefin/vinyl acetate (3:1) (M.W. 27,000) | 1       |
|    | Base oil blend (D)                                                                 | Balance |

|    |                                                                |         |
|----|----------------------------------------------------------------|---------|
| 60 | Composition IX:                                                |         |
|    | 1-hydroxyethyl-2-heptadecenyl imidazoline N-stearoyl sarcosine | 0.2     |
|    | Sodium petroleum sulfonate                                     | 0.6     |
|    | Base oil blend (A)                                             | Balance |

|    |                                   |         |
|----|-----------------------------------|---------|
| 65 | Composition X:                    |         |
|    | Octadecylamine N-oleoyl sarcosine | 0.1     |
|    | N-oleoyl sarcosine                | 0.1     |
|    | Sodium petroleum sulfonate        | 0.3     |
|    | Base oil blend (C)                | Balance |

The effectiveness of compositions of the present invention as high-speed quenching oils producing excellent surface finishes is demonstrated by testing such compositions as Compositions I, II and V and comparative Composition Z (base oil blend A+0.6% sodium petroleum sulfonate) and Composition Y (base oil blend A+0.6% N-oleoyl sarcosine) in the General Motors Magnetic Quench Test for Quenching Steel and Quenched Metal

Brightness described in The American Society for Metals bulletin on "Quenching of Steels," October 27-31, 1958, pages 29-42, wherein the brightness rating ranges from A to E with A being excellent and E being poor. Thus for Compositions Z and Y the brightness rating is E and A respectively, whereas for Compositions I, II and V the brightness rating is A and the quenching speed of Compositions I, II and V was equal to that of Composition Z, or improved by about 15% over Composition Y.

Compositions III, IV and VI to X also are excellent quenching speed oils and leave the surface metal clean and bright for further processing.

This application is a continuation-in-part of our co-pending application Serial No. 64,288, filed October 24, 1960, now U.S. Patent No. 3,112,232.

We claim as our invention:

1. A quenching oil composition consisting essentially of a mineral oil blend containing from 0.1 to 2% each of (A) an oil-soluble N—C<sub>10-24</sub> acyl sarcosine and (B) an oil-soluble metal petroleum sulfonate selected from the group consisting of alkali metal petroleum sulfonate and alkaline earth metal petroleum sulfonate, said blend consisting of a predominant amount of a high viscosity index oil having an aromatic content of from 20 to 60% and the balance of the blend being selected from the group consisting of a light oil having a viscosity range of from 40 to 100 SUS at 100° F., a heavy residue fraction having a viscosity of 150-210 and mixtures thereof.

2. The composition of claim 1 wherein the oil blend consists of a mixture of from 50-95% of 80-250 SUS at 100° F. HVI neutral oil having an aromatic content of from 20-60% and the balance being a bright stock.

3. The composition of claim 1 wherein the oil blend consists of a mixture of from 50-95% of 80-250 SUS at 100° F. HVI neutral oil having an aromatic content of from 20-60% and the balance being a propane asphalt.

4. The composition of claim 1 wherein the oil blend consists of a mixture of from 50-95% of 80-250 SUS at 100° F. HVI neutral oil having an aromatic content of from 20-60% and the balance being a spray base oil.

5. The composition of claim 1 wherein the oil blend consists of a mixture of from 50-95% of 80-250 SUS at 100° F. HVI neutral oil having an aromatic content

of from 20-60% and the balance being a refined transformer oil.

5 6. A quenching oil composition consisting of a mixture of from 50-95% of 80-250 SUS at 100° F. HVI neutral mineral oil having an aromatic content of from 30-60% and the balance being a mixture of bright stock and spray base oil, said mineral oil blend containing from 0.1 to 2% each of N-oleoyl sarcosine and sodium petroleum sulfonate.

10 7. A quenching oil composition consisting of a mixture of from 50-85% of 80-250 SUS at 100° F. HVI neutral mineral oil having an aromatic content of from 30-60% and the balance being a mixture of bright stock and spray base oil, said mineral oil blend containing from 0.1 to 2% 15 each of octadecyl amine salt of N-oleoyl sarcosine and sodium petroleum sulfonate.

20 8. A quenching oil composition consisting of a mixture of from 50-85% of 80-250 SUS at 100° F. HVI neutral mineral oil having an aromatic content of from 30-60% and the balance being a mixture of bright stock and spray base oil, said mineral oil blend containing from 0.1 to 2% 25 each of 1-hydroxyethyl-2-heptadecenyl imidazoline salt of N-oleoyl sarcosine and sodium petroleum sulfonate.

25 9. The composition of claim 6 containing a small amount of a polymeric dispersant and a phenolic antioxidant.

30 10. The composition of claim 8 containing a small amount of a polymeric dispersant and a phenolic antioxidant.

#### References Cited by the Examiner

##### UNITED STATES PATENTS

|    |           |       |                      |        |
|----|-----------|-------|----------------------|--------|
| 35 | 2,536,403 | 1/51  | Wallace et al. ----- | 148-29 |
|    | 2,670,310 | 2/54  | Freeman -----        | 148-28 |
|    | 2,799,606 | 7/57  | Freeman -----        | 148-28 |
|    | 3,112,232 | 11/63 | Early et al. -----   | 148-29 |

40 BENJAMIN HENKIN, Primary Examiner.

DAVID L. RECK, WINSTON A. DOUGLAS,

Examiners.